

# United States Patent Office

3,150,969

Patented Sept. 29, 1964

1

3,150,969

## BERYLLIUM-BRONZE ALLOY

Ellsworth M. Smith, Reading, Pa., assignor to The Brush Beryllium Company, Cleveland, Ohio, a corporation of Ohio

No Drawing. Filed Dec. 17, 1962, Ser. No. 244,862

3 Claims. (Cl. 75—153)

This invention relates generally to beryllium-copper alloys, and more particularly to beryllium-copper alloys containing zinc, cobalt, and optionally tin.

Hereinafter, all reference to percentages of ingredients are percentages of the total weight of the compositions.

It has been well established in the beryllium-copper alloy art that copper-based alloys containing beryllium and minor proportions of either cobalt, nickel, or mixtures thereof, upon being cold worked, as by rolling, and subsequently solution annealed, quenched, and heat treated in a temperature range of about 600° F. to about 800° F., developed high tensile strength, excellent fatigue endurance, excellent wear resistance, and good electrical conductivity. Such properties make possible the use of the alloys for springs, electrical contact components, welding rods, and the like. These desirable properties are imparted to the copper by incorporating therewith from about 1% to about 2% beryllium metal, and in addition, about 0.20% to about 0.40% of either cobalt or nickel, or mixtures thereof.

Known alloys of commercial importance in the beryllium-copper alloy art are copper based, and contain about 2% beryllium metal, and about 0.20% to about 0.40% of either cobalt or nickel, or mixtures thereof.

Because of the high cost of these commercial alloys, it has long been an objective of many workers in the beryllium-copper alloy art to obtain the mechanical properties of these known alloys while partially replacing the expensive beryllium metal content with other suitable and less expensive metals capable of producing such properties in the alloy.

Various metals have been employed as partial substituents for the beryllium metal content, such as nickel, cobalt, zinc, silver, aluminum, and magnesium, but the mechanical properties of the alloys when thus modified are not comparable to those of the known commercial alloys referred to above.

In a later development in the art, a beryllium-copper alloy containing about 1% beryllium was produced. This decrease of about 50% in the beryllium content of prior alloys was accomplished by replacing one half of the original 2% beryllium content with zinc. Since beryllium metal is the most expensive component of beryllium copper alloys, this development constituted a great advance in the art, particularly from an economic standpoint. The alloy containing 1% beryllium metal is disclosed and claimed in Donachie U.S. Patent No. 2,789,899, issued April 23, 1957.

In the file of the patent, the zinc content is said to be a matrix hardener for the copper and effective in amounts up to about 3.5%, by weight, of the composition. It is described as having no substantial effect upon the properties of the alloys in amounts above 3.5%, although some minor effect is shown from amounts of 3.5% up to about 5%.

Alloys having a beryllium content of less than 1%, by weight, of the composition, and retaining the same desirable mechanical properties as said commercial alloy have been proposed, but none of them has been found

2

to have mechanical properties comparable to those of the alloys containing 1% or 2% of beryllium.

The alloys of the present invention contain more than 10% and as high as about 25% zinc, from about a trace to about 1.00% tin, and metal from the class consisting of cobalt, nickel, and mixtures thereof, about 0.10% to about 0.40%. These additions have made possible a reduction in beryllium metal content to a range between about 0.30% and 1.0%, while providing the mechanical properties comparable to those of commercial alloys containing from about 1.0% to about 2.0% beryllium.

Whenever quantities of cobalt are specified in the alloy composition, nickel, its well-known equivalent, may be employed instead, in whole or part.

15 It is an object of this invention to provide a copper-based alloy containing beryllium, zinc, and optionally small proportions of tin and either cobalt or nickel, the alloy having mechanical properties, including age hardening characteristics, comparable to the commercial 20 alloys containing from about 1% to about 2% beryllium metal.

It is a further object of the invention to provide cold worked, solution annealed, quenched, and age hardened copper-based alloys containing less than 1% beryllium, 25 between about 10% and about 25% zinc, and minor amounts of tin and either cobalt or nickel, or mixtures thereof, and optionally tin in small amounts, said alloys having mechanical properties comparable to age-hardenable commercial alloys containing from about 1% up to 30 about 2% beryllium.

It is a still further object of the invention to provide such copper-based alloys having tensile and elongation properties superior to those specified for Phosphor bronze.

Another object is to provide alloys of the above composition which are capable of being rolled, drawn, extruded, forged, and pressed, by known techniques, without deterioration of their original mechanical properties.

The alloys of the present invention offer a further advantage in that when certain kinds of metal scrap are employed in producing the composition, the method of combining the various metallic components to provide the final composition does not require rigid control, because the components of the scrap, generally considered undesirable for alloys of optimum mechanical properties, are beneficial as metal components of the present alloy.

These and other objects and advantages of the invention will be obvious from the following description.

The essential constituents of the present alloys are broadly the following:

|    | Range, weight percent |
|----|-----------------------|
| Be | 0.30-1.10             |
| Co | 0.07-0.40             |
| Zn | 10.00-25.00           |
| Sn | Trace-1.00            |
| Cu | Balance               |

More specifically, the alloys fall within the following range:

|    | Range Weight, percent | Preferred Wt., percent |
|----|-----------------------|------------------------|
| Be | 0.65-0.85             | 0.75                   |
| Co | 0.10-0.30             | 0.20                   |
| Zn | 15.00-20.00           | 17.50                  |
| Sn | Trace-0.85            | 0.25                   |
| Cu | Balance               | Balance                |

Tin in amounts of from a trace to about 1.00% often unavoidably introduced as part of the scrap added to the charge, has no deleterious effect on the mechanical properties of the alloy. However, it is desirable to maintain the tin in a range from about a trace to about 0.85%, as alloys containing more than about 0.85%, although possessing satisfactory mechanical properties, are not as amenable to fabrication operations. Also, when the tin content is more than about 1.5%, ingots of such composition tend to edge crack when rolled into strip.

The alloys may be produced by the conventional manner of melting a predetermined quantity of the elemental metals and casting the melt into ingots, or by any other conventional method of producing alloys. When prepared in a melt, the cast ingots may then be fabricated by conventional methods into sheets, bars, tubes, and wire.

In Table I below, examples of the alloy compositions and the mechanical properties developed by solution annealing and various degrees of cold working and heat treatment are shown. The test data were obtained from strip which, in the solution annealed form, was 0.020" in thickness. To obtain the strip, a melt of predetermined quantities of the elemental metals was prepared and cast into ingots, which were first hot rolled and then cold rolled to a thickness of 0.09" and solution annealed. The annealed strip of this thickness was then cold rolled in five passes to a thickness of 0.020", strand annealed at 1450° F. for about 1.5 minutes, and quenched in water. The strip was then strand pickled, slit into sections, one of which was tested in the annealed condition, and the others cold rolled to various degrees of reduced thickness and heat treated as shown in the table.

The examples presented in the table show that the alloys containing from 0.65% to 0.85% beryllium and from about 15% to about 20% of zinc in the solution annealed and heat treated or age hardened conditions have properties comparable to those of the commercial beryllium-copper alloys containing from 1% to about 2% beryllium, and have superior mechanical properties to Phosphor bronze of the commercial grade A and spring temper types.

The expression "balance substantially copper," as employed in the appended claims, does not exclude small quantities of addition metals or metal impurities, such as aluminum, silver, and magnesium, in proportions insufficient to substantially change the characteristics or mechanical properties of the said alloys.

TABLE I  
Compositions and Mechanical Properties of Beryllium-Bronze Alloys

| Alloy | Chemical Composition, Weight Percent |      |      |       |      | Temper <sup>a</sup> | Mechanical Properties             |                          |
|-------|--------------------------------------|------|------|-------|------|---------------------|-----------------------------------|--------------------------|
|       | Be                                   | Co   | Zn   | Sn    | Cu   |                     | Ultimate Tensile Strength, p.s.i. | Percent Elongation in 2" |
| A     | 0.32                                 | 0.32 | 11.0 | 0.22  | Bal. | Ann.                | 51,700                            | 40                       |
|       |                                      |      |      |       |      | AT                  | 53,000                            | 40                       |
|       |                                      |      |      |       |      | 1/2 H               | 66,500                            | 12                       |
|       |                                      |      |      |       |      | 1/2 HT              | 71,000                            | 20                       |
|       |                                      |      |      |       |      | XH                  | 90,000                            | 2                        |
|       |                                      |      |      |       |      | XHT                 | 91,000                            | 9                        |
| B     | 0.56                                 | 0.15 | 20.6 | 0.35  | Bal. | Ann.                | 66,700                            | 50                       |
|       |                                      |      |      |       |      | AT                  | 106,500                           | 22                       |
|       |                                      |      |      |       |      | 1/2 H               | 79,500                            | 28                       |
|       |                                      |      |      |       |      | 1/2 HT              | 113,000                           | 7                        |
|       |                                      |      |      |       |      | XH                  | 111,000                           | 2                        |
|       |                                      |      |      |       |      | XHT                 | 140,500                           | 1                        |
| C     | 0.51                                 | 0.36 | 20.7 | <0.01 | Bal. | Ann.                | 72,000                            | 40                       |
|       |                                      |      |      |       |      | AT                  | 103,000                           | 19                       |
|       |                                      |      |      |       |      | 1/2 H               | 91,000                            | 18                       |
|       |                                      |      |      |       |      | 1/2 HT              | 129,000                           | 7                        |
|       |                                      |      |      |       |      | H                   | 109,000                           | 4                        |
|       |                                      |      |      |       |      | HT                  | 144,000                           | 2                        |
| D     | 0.58                                 | 0.30 | 15.8 | 0.48  | Bal. | Ann.                | 66,000                            | 53                       |
|       |                                      |      |      |       |      | AT                  | 105,500                           | 26                       |
|       |                                      |      |      |       |      | 1/2 H               | 83,000                            | 23                       |
|       |                                      |      |      |       |      | 1/2 HT              | 123,000                           | 18                       |
|       |                                      |      |      |       |      | XH                  | 110,000                           | 2                        |
|       |                                      |      |      |       |      | XHT                 | 144,500                           | 4                        |

<sup>a</sup> NOTE.—The following schedule defines the temper designations used throughout Table I:

Ann.—Solution annealed at 1450° F. for one and one-half minutes and quenched.

AT—Solution annealed at 1450° F. for one and one-half minutes, quenched, and heat treated at 600° F. for three hours.

1/2 H—Solution annealed at 1450° F. for one and one-half minutes, quenched, and reduced 20% in thickness by cold rolling.

1/2 HT—Solution annealed at 1450° F. for one and one-half minutes, quenched, reduced 20% in thickness by cold rolling, and heat treated at 600° F. for three hours.

H—Solution annealed at 1450° F. for one and one-half minutes, quenched, and reduced 40% in thickness by cold rolling.

HT—Solution annealed at 1450° F. for one and one-half minutes, quenched, reduced 40% in thickness by cold rolling, and heat treated at 600° F. for 3 hrs.

XH—Solution annealed at 1450° F. for one and one-half minutes, quenched, reduced 50% in thickness by cold rolling.

XHT—Solution annealed at 1450° F. for one and one-half minutes, quenched, reduced 50% in thickness by cold rolling, and heat treated at 600° F. for 3 hrs.

Having thus described my invention, I claim:

- An alloy consisting essentially of about 0.30% to about 1.10% of beryllium, about 0.10% to about 0.40% of metal from the group consisting of cobalt, nickel, and mixtures thereof, about 9% to about 25% of zinc, a trace

to about 1.0% of tin, and the balance essentially copper.

2. An alloy consisting essentially of about 0.65% to about 0.85% of beryllium, about 0.10 to about 0.30% of metal from the class consisting of cobalt, nickel and mixtures thereof, a trace to about 0.85% of tin, about 15% to about 20% of zinc, and the balance essentially copper.

3. An alloy consisting essentially of beryllium about 0.75%, cobalt about 0.20%, zinc about 17.5%, tin about 0.25%, and the balance essentially copper.

5

10 521,731

**References Cited in the file of this patent****UNITED STATES PATENTS**

|           |                |       |               |
|-----------|----------------|-------|---------------|
| 2,145,625 | Kinzel         | ----- | Jan. 31, 1939 |
| 2,412,447 | Donachie       | ----- | Dec. 10, 1946 |
| 2,422,477 | Driver         | ----- | June 17, 1947 |
| 2,783,143 | Johnson et al. | ----- | Feb. 26, 1957 |
| 2,789,899 | Donachie       | ----- | Apr. 23, 1957 |

**FOREIGN PATENTS**

|               |       |              |
|---------------|-------|--------------|
| Great Britain | ----- | May 29, 1940 |
|---------------|-------|--------------|